

2,798,018

## METHOD OF REMOVING GASEOUS SEGREGATION FROM METALS

Gerhard Derge, Aspinwall, Pa., assignor to Carnegie Institute of Technology, Pittsburgh, Pa., a corporation of Pennsylvania

No Drawing. Application September 29, 1952,  
Serial No. 312,170

20 Claims. (Cl. 148—13)

This invention relates to the removal of gaseous segregation from metal objects and particularly to the removal of hydrogen segregation from ferrous metal objects. The presence of gases in metals is generally known to produce inferior physical properties which in turn result in unacceptable behavior or failure in the finished product fabricated from such metals.

One of the most familiar examples of gaseous segregation in metals is hydrogen segregation in steel and other ferrous metal objects. The presence of hydrogen in steel results in several undesirable physical conditions. One of the most common conditions associated with the presence of hydrogen is the formation of what are commonly termed "flakes." These are small internal ruptures within the steel itself. Flakes frequently occur midway between the surface of the steel and the center of a section and are particularly undesirable in the finished product since there is nothing that can be done about them once the object has reached its final finished form. Hydrogen also has a very undesirable embrittling effect upon steel in which it occurs. As in the case of formation of "flakes," the nature of this embrittling effect is not completely understood, however, steels in which hydrogen is present in substantial amounts show low ductility and other characteristics of embrittlement. All of these characteristics are generally undesirable in steel products. There has, however, been no way of positively controlling the segregation of hydrogen or other gases in steel and other metals. The only existing commercial practices which seem to reduce the undesirable effects which result from the presence of hydrogen are either to subject the product to special heat treatments or to very slow cooling cycles. Both of these methods are expensive because they tie up equipment and materials for inconveniently long periods of time—often as long as several days.

I have discovered a method by means of which gaseous segregation in metal objects can be substantially removed and the gases remaining in the metal object distributed substantially homogeneously throughout the object. In a preferred practice of my invention I follow the steps of uniformly heating a portion of a solid metal body from which gaseous segregation is to be removed, advancing the zone of maximum temperature along the body and permitting progressive cooling of the before heated portions during such progression. The progression is carried out at a controlled rate whereat a substantial portion of the gas content migrates with the advancement of the heated zone. The rate of progression will vary depending upon the conditions, e. g., temperature, composition of the body, etc., however, once conditions are established for a particular body the rate is substantially constant from body to body.

I have found that the method of my invention may be carried out effectively by passing the object through a heated zone into a cooler zone so that the portion of the object in the heated zone is always at a higher temperature than the adjoining portion of the object in the

cooler zone and so that the last-heated portion includes an external surface or a portion which is subsequently to be removed from the object, maintaining the last-heated portion at the heating temperature until the balance of the object is substantially lower in temperature and then removing the last-heated portion from the heated zone into the cooler zone.

I have found that the method of my invention is particularly satisfactory for the removal of hydrogen from steel and is most effective for this purpose when the heated portions of the steel object are in the austenitic region. I have found that by following this method hydrogen may be moved at least 4 inches in less than 15 minutes by heating and then quenching a steel test piece from one end. For example, a modified Jominy test piece was heated to approximately 1600° F. One end of the heated test piece was then quenched by spraying the end face with cooling liquid. The hydrogen moved through the test piece from the quenched end as the piece cooled and migrated to the portion which was held above 1000° F. for the greatest period of time. The results of this treatment are tabulated in Table I below.

Table I

| Sample No. | Distance Quenched End | Percent H | Time Above 1,000° F. in Minutes |
|------------|-----------------------|-----------|---------------------------------|
| 1          | 0.5                   | .000014   | 1.0                             |
| 2          | 1.5                   | .000016   | 2.5                             |
| 3          | 2.5                   | .000020   | 5.0                             |
| 4          | 3.5                   | .000038   | 9.0                             |
| 5          | 4.0                   | .000049   | 10.0                            |

The opposite end of the test piece was permitted to air-cool and a similar migration away from the air-cooled end was noted.

| Sample No. | Distance Air-Cooled End | Percent H | Time Above 1,000° F. in Minutes |
|------------|-------------------------|-----------|---------------------------------|
| 8          | 0.5                     | .000021   | 7.0                             |
| 7          | 1.5                     | .000030   | 10.0                            |
| 6          | 2.0                     | .000035   | 10.5                            |

The method of this invention is preferably carried out commercially by progressively removing an object being treated from a furnace in which it has been heated. For example, a billet of steel 10 inches in diameter and 15 feet long can be removed progressively from a furnace maintained in the austenitic temperature range at the rate of about 3 feet per hour and the hydrogen will be evenly distributed at a low concentration in all but the last few feet of the billet which is normally cropped. It is possible to remove the hydrogen from the last few feet if the timing of the withdrawal is correct, that is if the last few feet are retained at the furnace temperature until the hydrogen diffuses into the atmosphere.

The method of this invention may also be carried out by progressively passing an object to be treated through a furnace and into a cooling zone so that the portion leaving the furnace and entering the cooling zone is in contact with a portion within the furnace having a temperature substantially equal to or above that of the portion leaving the furnace.

In any practice of my invention it is of course obvious that the rate of heating and the rate of cooling must be regulated to suit the particular metal object being processed. For example, heating must be regulated to prevent warping or distortion, etc. in the finished piece while at the same time assuring a uniform temperature in the heated portion of the object.

The method of my invention appears to be based upon a "flow" of gas e. g. hydrogen, from a cooling portion to a portion of higher temperature as if from a place of higher to one of lower potential. This results in a metal object in which a substantial amount of the gases are removed while the remaining gases are substantially homogeneously distributed throughout the ingot from side to side as well as from end to end.

While I have described the preferred practices of my invention it will be understood that it may be otherwise practiced within the scope of the following claims.

I claim:

1. A method of removing gaseous segregation from a solid metal object having gaseous segregation while in said solid state, comprising the steps of heating the object while retaining the object in the solid state and successively cooling adjoining portions of the heated object so that the last-cooled portion includes an external surface while maintaining said last-cooled portion at the heating temperature until the gases have substantially diffused therefrom to the atmosphere.

2. A method of removing gaseous segregation from a solid metal object having gaseous segregation while in said solid state, comprising the steps of passing the object through a heated zone into a cooler, all the while retaining the object in the solid state, maintaining the last-heated portion at the heating temperature until the balance of the object is substantially lower in temperature and until the gases have substantially diffused from the last-heated portion to the atmosphere and removing the last-heated portion from the heated zone to the cooler zone.

3. A method of removing gaseous segregation from a solid metal object having gaseous segregation while in said solid state, comprising the steps of passing the object through a heated zone into a cooler zone so that the portion of the object in the heated zone is always at a higher temperature than the adjoining portion of the object in the cooler zone and so that the last-heated portion includes an external surface, all the while maintaining the object in the solid state, maintaining the last-heated portion at the heating temperature until the balance of the object is substantially lower in temperature and until the gases have substantially diffused from the last-heated portion to the atmosphere, and then removing the last-heated portion from the heated zone into the cooler zone.

4. A method of removing gaseous segregation from a solid metal object having gaseous segregation while in said solid state, comprising the steps of forming the object with a portion to be subsequently removed, passing the object through a heated zone into a cooler zone so that the portion to be removed is the last portion to pass into the cooler zone, all the while retaining the object in the solid state, maintaining the portion to be removed at the heating temperature until the balance of the object is substantially lower in temperature, removing said portion from the heated zone and removing said portion from the object.

5. A method of removing hydrogen from a solid steel object having hydrogen segregation while in the solid state, comprising the steps of heating the steel object while retaining it in the solid state and successively cooling adjoining portions thereof so that the last-cooled portion includes an external surface while maintaining said last-cooled portion at the heating temperature until the hydrogen has substantially diffused therefrom to the atmosphere.

6. A method of removing hydrogen from a solid steel object having hydrogen segregation while in the solid state, comprising the steps of passing the object through a heated zone into a cooler zone, all the while retaining the object in the solid state, maintaining the last-heated portion at the heating temperature until the balance of the object is substantially lower in temperature and until the hydrogen has substantially diffused therefrom to the

atmosphere, and removing the last-heated portion from the heated zone to the cooler zone.

5 7. A method of removing hydrogen from a solid steel object having hydrogen segregation while in the solid state, comprising the steps of passing the object through a heated zone into a cooler zone so that the portion of the object in the heated zone is always at a higher temperature than the adjoining portion of the object in the cooler zone and so that the last-heated portion includes an external surface, all the while retaining the object in the solid state, maintaining the last-heated portion at the heating temperature until the balance of the object is substantially lower in temperature and until the hydrogen has substantially diffused therefrom to the atmosphere, and then removing the last-heated portion from the heated zone into the cooler zone.

10 8. The method of removing hydrogen from a solid steel object having hydrogen segregation while in the solid state, comprising the steps of forming the object with a portion to be subsequently removed, passing the object through a heated zone into a cooler zone so that the portion to be removed is the last portion to pass into the cooler zone, all the while retaining the object in the solid state, maintaining the portion to be removed at the heating temperature until the balance of the object is substantially lower in temperature, removing said portion from the heated zone and removing said portion from the object.

15 9. The method of removing gaseous segregation from a solid steel object having gaseous segregation while in said solid state, comprising the steps of heating the object to the austenitic region, all the while retaining the object in the solid state, and successively cooling adjoining portions of the heated object so that the last-cooled portion includes an external surface while maintaining said last-cooled portion in the austenitic region until the gases have substantially diffused therefrom to the atmosphere.

20 10. The method of removing gaseous segregation from a solid steel object having gaseous segregation while in said solid state, comprising the steps of passing the object through a heated zone to raise its temperature to the austenitic region, all the while retaining the object in the solid state, passing the object into a cooler zone, maintaining the last-heated portion in the austenitic temperature region until the balance of the object is substantially lower in temperature and until the gases have substantially diffused from the last-heated portion to the atmosphere, and removing the last-heated portion from the heated zone to the cooler zone.

25 11. A method of removing gaseous segregation from a solid steel object having gaseous segregation while in said solid state, comprising the steps of passing the object through a heated zone to raise its temperature to an austenitic region, all the while retaining the object in the solid state, passing the object into a cooler zone at a rate such that the portion of the object in the heated zone is always at a higher temperature than the adjoining portion of the object in the cooler zone and so that the last-heated portion includes an external surface, maintaining the last-heated portion in the austenitic temperature region until the balance of the object is substantially lower in temperature and until the gases have substantially diffused from the last-heated portion to the atmosphere, and removing the last-heated portion from the heated zone to the cooler zone.

30 12. A method of removing a gaseous segregation from a solid steel object having gaseous segregation while in said solid state, comprising the steps of forming the object with a portion to be subsequently removed, passing the object through a heated zone to raise its temperature to the austenitic region, all the while retaining the object in the solid state, passing the object into a cooler zone in such manner that the portion to be removed is the last portion to pass into the cooler zone, maintaining the por-

tion to be removed in the austenitic temperature region until the balance of the object is substantially lower in temperature, cooling said last-heated portion and removing it from the object.

13. The method of removing hydrogen from a solid steel object having hydrogen segregation while in the solid state, comprising the steps of heating the object to the austenitic region, all the while retaining the object in the solid state, and successively cooling adjoining portions of the heated object so that the last-cooled portion includes an external surface while maintaining said last-cooled portion at the heating temperature until the hydrogen has substantially diffused therefrom to the atmosphere.

14. The method of removing hydrogen from a solid steel object having hydrogen segregation while in the solid state, comprising the steps of passing the object through a heated zone to raise its temperature to the austenitic region, all the while retaining the object in the solid state, passing the object into a cooler zone, maintaining the last-heated portion in the austenitic temperature region until the balance of the object is substantially lower in temperature and until the hydrogen has substantially diffused therefrom to the atmosphere, and removing the last-heated portion from the heated zone to the cooler zone.

15. The method of removing hydrogen from a solid steel object having hydrogen segregation while in the solid state, comprising the steps of passing the object through a heated zone to raise its temperature to the austenitic region, all the while retaining the object in the solid state, passing the object into a cooler zone at a rate such that the portion of the object in the heated zone is always at a higher temperature than the adjoining portion of the object in the cooler zone and so that the last-heated portion includes an external surface, maintaining the last-heated portion in the austenitic temperature region until the balance of the object is substantially lower in temperature and until the hydrogen has substantially diffused therefrom to the atmosphere, and removing the last-heated portion from the heated zone to the cooler zone.

16. The method of removing hydrogen from a solid steel object having hydrogen segregation while in the solid state, comprising the steps of forming the object with a portion to be subsequently removed, passing the object through a heated zone to raise its temperature to the austenitic region, all the while retaining the object in the solid state, passing the object into a cooler zone in such manner that the portion to be removed is the last portion to pass into the cooler zone, maintaining the portion to be removed in the austenitic temperature region until the balance of the object is substantially lower in temperature, cooling said last-heated portion and removing it from the object.

17. A method of reducing gaseous segregation in solid metal bodies having gaseous segregation while in said solid state, comprising locally heating a portion of the body, advancing the zone of maximum temperature along the body, all the while retaining the object in the solid state, and permitting progressive cooling of the before heated portions during such progression, the progression

being at a controlled rate whereat a substantial portion of the gas content migrates with the advancement of the heated zone and maintaining the last-heated zone at the maximum temperature until the gases have substantially diffused to the atmosphere.

18. A method of reducing gaseous segregation in solid metal bodies having gaseous segregation while in said solid state, comprising locally heating a portion of the body while an adjacent portion of the body is at a lesser temperature, advancing the zone of maximum temperature along the body, all the while retaining the object in the solid state, and permitting progressive cooling of the before heated portions during such progression, the progression being at a controlled rate whereat a substantial portion of the gas content migrates with the advancement of the heated zone and maintaining the last heated zone at the maximum temperature until the gases have substantially diffused to the atmosphere.

19. The method of reducing hydrogen content of solid ferrous bodies having hydrogen segregation while in said solid state, comprising locally heating a portion of the body to the austenitic region, advancing the zone of maximum temperature along the body, all the while retaining the object in the solid state, and permitting progressive cooling of the before heated portions during such progression, the progression being at a controlled rate whereat a substantial portion of the gas content migrates with the advancement of the heated zone and maintaining the last heated portion of the body in the austenitic region until the gases have substantially diffused to the atmosphere.

20. A method of reducing hydrogen content of solid ferrous bodies having hydrogen segregation while in said solid state, comprising locally heating a portion of the body to the austenitic region while an adjacent portion of the body is at a lesser temperature, advancing the zone of maximum temperature of the body, all the while retaining the body in the solid state, and permitting progressive cooling of the before heated portions during such progression, the progression being at a controlled rate whereat a substantial portion of the gas content migrates with the advancement of the heated zone and maintaining the last heated portion in the austenitic region until the gases have substantially diffused to the atmosphere.

#### 45 References Cited in the file of this patent

##### UNITED STATES PATENTS

|              |          |                |
|--------------|----------|----------------|
| 1,732,244    | Salzman  | Oct. 22, 1929  |
| 1,733,752    | Ramage   | Oct. 29, 1929  |
| 50 1,738,307 | McKeehan | Dec. 3, 1929   |
| 1,980,875    | Northrop | Nov. 13, 1934  |
| 2,131,062    | McBride  | Sept. 27, 1938 |
| 2,417,094    | Spinasse | Mar. 11, 1947  |
| 2,739,088    | Pfann    | Mar. 20, 1956  |

##### 55 FOREIGN PATENTS

|           |        |               |
|-----------|--------|---------------|
| 1,065,523 | France | Jan. 13, 1954 |
|-----------|--------|---------------|

##### 60 OTHER REFERENCES

Metals Handbook, 1948, p. 1208.

UNITED STATES PATENT OFFICE  
CERTIFICATE OF CORRECTION

Patent No. 2,798,018

July 2, 1957

Gerhard Derge

It is hereby certified that error appears in the printed specification of the above numbered patent requiring correction and that the said Letters Patent should read as corrected below.

Column 2, line 39, Table I, fourth column thereof, in the heading, line 2, for "1,000 F." read -- 1,000° F. --; column 3, line 25, after "cooler" and before the comma insert -- zone --; column 6, line 51, list of references cited, under the heading "UNITED STATES PATENTS" for "Northrop" read -- Northrup --.

Signed and sealed this 29th day of October 1957.

(SEAL)

Attest:

KARL H. AXLINE

Attesting Officer

ROBERT C. WATSON  
Commissioner of Patents